

## UNITED STATES PATENT OFFICE

2,596,221

## PROCESS OF YARN MANUFACTURING

Robert G. Dort, Summit, N. J., assignor to Celanese Corporation of America, New York, N. Y., a corporation of Delaware

No Drawing. Application April 7, 1950,  
Serial No. 154,741

8 Claims. (Cl. 57—157)

1

This invention relates to yarns and relates more particularly to heavy denier, continuous filament yarns suitable for the production of carpeting, heavy upholstery fabrics and similar textile materials.

As is well known, the heavy denier yarns that are employed for the production of carpeting, heavy upholstery fabrics and similar textile materials must exhibit a high degree of resilience so that they will regain their shape after being placed under load. These heavy denier yarns must also show little tendency toward matting which would rapidly destroy the usefulness of the materials produced therefrom. When heavy denier yarns are employed for the production of carpeting, heavy upholstery fabrics and similar textile materials having a cut pile, the yarns must have the ability to bloom or expand so that the cut pile will present a desirable uniform appearance. In addition, the heavy denier yarns must be uniform throughout their cross-section and must be easily handled both during the manufacture, dyeing and other processing thereof and during the production of carpeting, heavy upholstery fabric and similar textile materials therefrom.

Heretofore, it has been the general practice to prepare heavy denier yarns suitable for the production of carpeting, heavy upholstery fabrics and similar textile materials from natural fibers or from synthetic fibers of staple length. As will be readily apparent, there is a considerable expense involved in converting the natural fibers or synthetic fibers of staple length into yarns, which expense increases the cost of the materials produced from said yarns.

It is an important object of this invention to provide a process for the manufacture of heavy denier yarns suitable for the production of carpeting, heavy upholstery fabrics and similar textile materials that will be free from the foregoing and other disadvantages of the processes previously used for this purpose.

A further object of this invention is the provision of an efficient and inexpensive process for the manufacture of heavy denier, continuous filament yarns suitable for the production of carpeting, heavy upholstery fabrics and similar textile materials.

Other objects of this invention will be apparent from the following detailed description and claims.

I have now discovered that the expense involved in converting natural fibers or synthetic fibers of staple length into heavy denier yarns

2

suitable for the production of carpeting, heavy upholstery fabrics and similar textile materials may be eliminated by manufacturing said heavy denier yarns from continuous filaments. According to the present invention, a large number of continuous filaments are assembled in substantially parallel relation to form a tow having a total denier of between about 1,000 and 10,000. The individual filaments going into said tow may have a denier of between about 3 and 40 to produce yarns suitable for conversion into carpeting, heavy upholstery fabrics and similar textile materials of all weights and types. It is, however, preferred to keep the denier of the individual filaments between about 8 and 20, it having been found that filaments of this denier produce yarns possessing the most desirable characteristics. The individual filaments are preferably assembled into a tow in the spinning apparatus in which they are formed or immediately after they leave such spinning apparatus.

The tow is treated so as to impart a crimp to the individual filaments contained therein. Crimping may be effected by passing the tow through a stuffing box, between a pair of crimping rollers or by any other mechanical means that will distort the individual filaments under a sufficient pressure to impart a permanent set thereto. Advantageously, the tow is flattened to form a ribbon of continuous filaments before it is passed through the crimping mechanism so that all the filaments will have a crimp imparted thereto.

It is essential that the continuous filaments be in substantially parallel relation and extend along the length of the tow during the crimping operation. If the tow has any appreciable twist therein, or if the continuous filaments are not in substantially parallel relation, the superficial filaments of the tow will act as a cushion to limit the effect of the crimping mechanism on the inner filaments of the tow and these inner filaments will receive little or no crimp. A tow containing filaments having little or no crimp will not be suitable for the production of heavy denier yarns. The crimp increases the resilience of the continuous filaments and also the ability of the yarns containing the same to bloom or expand when they are employed for the production of a cut pile. The crimp also improves the handling properties of the tow, preventing the individual filaments from tangling one with the other and from separating completely from the tow.

Following the crimping operation, a twist of 55 from about 2 to 12 turns per inch is applied to

the tow converting it into yarn. Twisting may be carried out on any textile apparatus suitable for the purpose such as a cap twister, a ring twister or the like. It is undesirable to put a twist higher than 12 turns per inch into the yarn since the high twist will impede the access of dyebaths and other processing solutions to the filaments lying at the center of the yarn. Similarly, it is undesirable to put a twist lower than 2 turns per inch into the yarn since such a low twist will permit individual filaments to be separated from the yarn during the dyeing and other processing thereof and during the production of carpeting, heavy upholstery fabrics and similar textile materials therefrom.

The yarns may be dyed to impart thereto any desired color and shade. Dyeing may be effected while the yarns are in the form of hanks or skeins, or while the yarns are wound onto perforated bobbins or the like. The dyed yarns are washed and dried and may then be employed for the production of carpeting, heavy upholstery fabrics and similar textile materials having either a loop pile or a cut pile.

The yarn produced in accordance with this invention may be used alone or they may be plied with from 1 to 7 other yarns having the same or a reverse twist and formed from natural fibers or from the same or different synthetic fibers. The plied yarn may have a twist of from 5 to 20 turns per inch therein. The filaments of all of the yarns that are plied one with the other may have a basis of an organic derivative of cellulose such as cellulose acetate, cellulose propionate, cellulose butyrate, cellulose acetate-propionate, cellulose acetate-butyrate, ethyl cellulose, benzyl cellulose or the like. Alternatively, yarns prepared in accordance with the process of this invention and composed of continuous filaments having a basis of an organic derivative of cellulose such as cellulose acetate may be plied with woolen or cotton yarns or with yarns having a basis of regenerated cellulose, such as viscose yarns. When plied yarns containing fibers of different composition are employed for the production of carpeting, heavy upholstery fabric and similar textile materials, these materials may be cross-dyed in a manner well known in the art to impart thereto a novel and unusual appearance.

The following example is given to illustrate this invention further.

*Example*

A large number of continuous filaments of cellulose acetate having a denier of 17 are assembled, as they leave the spinning apparatus in which they are formed, into a tow having a total denier of 2300. The tow is passed directly to a crimping apparatus wherein it is flattened to form a ribbon of continuous filaments and is passed through a crimping mechanism which imparts a crimp to all the filaments therein. The crimped tow is passed to a cap twister which inserts therein a twist of 4.5 turns per inch. The yarn produced in this manner shows a good resilience, little tendency toward matting and may, after dyeing, be employed for the production of carpeting, heavy upholstery fabrics and similar textile materials.

It is to be understood that the foregoing detailed description is given merely by way of illustration and that many variations may be made therein without departing from the spirit of my invention.

Having described by invention, what I desire to secure by Letters Patent is:

1. In a process for the manufacture of heavy denier yarns suitable for the production of carpeting, heavy upholstery fabrics and similar textile materials, the steps which comprise assembling a plurality of continuous unitary filaments in substantially parallel relation to form a tow having a total denier of between about 1,000 and 10,000, crimping all the filaments in the tow while the filaments are in substantially parallel relation in a single plane and extend along the length of the tow, and applying a twist to the tow of between about 2 and 12 turns per inch.

2. In a process for the manufacture of heavy denier yarns suitable for the production of carpeting, heavy upholstery fabrics and similar textile materials, the steps which comprise assembling a plurality of continuous unitary filaments having a denier between about 3 and 40 in substantially parallel relation to form a tow having a total denier of between about 1,000 and 10,000, crimping all the filaments in the tow while the filaments are in substantially parallel relation in a single plane and extend along the length of the tow, and applying a twist to the tow of between about 2 and 12 turns per inch.

3. In a process for the manufacture of heavy denier yarns suitable for the production of carpeting, heavy upholstery fabrics and similar textile materials, the steps which comprise assembling a plurality of continuous unitary filaments having a denier between about 8 and 20 in substantially parallel relation to form a tow having a total denier of between about 1,000 and 10,000, crimping all the filaments in the tow while the filaments are in substantially parallel relation in a single plane and extend along the length of the tow, and applying a twist to the tow of between about 2 and 12 turns per inch.

4. In a process for the manufacture of heavy denier yarns suitable for the production of carpeting, heavy upholstery fabrics and similar textile materials, the steps which comprise assembling a plurality of continuous filaments in substantially parallel relation to form a tow having a total denier of between about 1,000 and 10,000, flattening the tow to form a ribbon of continuous filaments, crimping all the filaments in the flattened tow while the filaments are in substantially parallel relation and extend along the length of the tow, and applying a twist to the tow of between about 2 and 12 turns per inch.

5. In a process for the manufacture of heavy denier yarns suitable for the production of carpeting, heavy upholstery fabrics and similar textile materials, the steps which comprise assembling a plurality of continuous filaments having a denier between about 8 and 20 in substantially parallel relation to form a tow having a total denier of between about 1,000 and 10,000, flattening the tow to form a ribbon of continuous filaments, crimping all the filaments in the flattened tow while the filaments are in substantially parallel relation and extend along the length of the tow, and applying a twist to the tow of between about 2 and 12 turns per inch.

6. In a process for the manufacture of heavy denier yarns suitable for the production of carpeting, heavy upholstery fabrics and similar textile materials, the steps which comprise assembling a plurality of continuous filaments having a basis of an organic derivative of cellulose and having a denier between about 8 and 20 in substantially parallel relation to form a tow having

a total denier of between about 1,000 and 10,000, flattening the tow to form a ribbon of continuous filaments, crimping all the filaments in the flattened tow while the filaments are in substantially parallel relation and extend along the length of the tow, and applying a twist to the tow of between about 2 and 12 turns per inch.

7. In a process for the manufacture of heavy denier yarns suitable for the production of carpeting, heavy upholstery fabrics and similar textile materials, the steps which comprise assembling a plurality of continuous filaments having a basis of cellulose acetate and having a denier between about 8 and 20 in substantially parallel relation to form a tow having a total denier of between about 1,000 and 10,000, flattening the tow to form a ribbon of continuous filaments, crimping all the filaments in the flattened tow while the filaments are in substantially parallel relation and extend along the length of the tow, and applying a twist to the tow of between about 2 and 12 turns per inch.

8. In a process for the manufacture of heavy denier yarns suitable for the production of

carpeting, heavy upholstery fabrics and similar textile materials, the steps which comprise assembling a plurality of continuous filaments having a basis of cellulose acetate and having a denier between about 8 and 20 in substantially parallel relation to form a tow having a total denier of between about 1,000 and 10,000, flattening the tow to form a ribbon of continuous filaments, crimping all the filaments in the flattened tow while the filaments are in substantially parallel relation and extend along the length of the tow, applying a twist to the tow of between about 2 and 12 turns per inch to convert the same to a yarn, and plying the yarn with other yarns.

ROBERT G. DORT.

#### REFERENCES CITED

The following references are of record in the file of this patent:

#### UNITED STATES PATENTS

| Number    | Name        | Date          |
|-----------|-------------|---------------|
| 2,356,887 | Rutishauser | Aug. 29, 1944 |